

# United States Patent

Yperman et al.

[15] 3,674,713

[45] July 4, 1972

[54] **ELECTRIC CERAMIC RESISTORS  
HAVING POSITIVE TEMPERATURE  
COEFFICIENTS AND METHOD OF  
MANUFACTURING SAME**

[72] Inventors: Jean Michel Baudry Ghislain yperman,  
Charles Belhomme, Evere, both of Belgium

[73] Assignee: U.S. Philips Corporation, New York, N.Y.

[22] Filed: Jan. 26, 1970

[21] Appl. No.: 6,052

**Related U.S. Application Data**

[63] Continuation of Ser. No. 601,343, Dec. 13, 1966,  
abandoned.

[30] **Foreign Application Priority Data**

Dec. 18, 1965 Netherlands.....6516534

[52] U.S. Cl. ....252/520, 106/39 R, 252/521  
[51] Int. Cl. ....H01c 7/02  
[58] Field of Search.....252/520, 62.1, 106/39 R

[56] **References Cited**

**UNITED STATES PATENTS**

2,515,790 7/1950 Navias.....106/63  
2,981,699 4/1961 Ichikawa.....252/520

*Primary Examiner*—Richard D. Lovering  
*Attorney*—Frank R. Trifari

[57] **ABSTRACT**

A barium titanate semiconductive resistor having a high positive temperature coefficient of electrical resistance and containing a small amount of a fluoride.

**8 Claims, No Drawings**

**ELECTRIC CERAMIC RESISTORS HAVING POSITIVE  
TEMPERATURE COEFFICIENTS AND METHOD OF  
MANUFACTURING SAME**

This application is a continuation of application Ser. No. 601,343, filed Dec. 13, 1966 and now abandoned.

The invention relates to a method of manufacturing ceramic resistance bodies for electric resistors having a positive temperature coefficient of the electric resistivity, which bodies mainly consist of semiconductive barium titanate; the invention further relates to resistance bodies thus manufactured and resistors manufactured by means of said bodies (so-called PTC-resistors).

The expression semiconductor ceramic resistance bodies on the basis of barium titanate is to be understood to mean hereinafter such bodies which have been made semiconductive with the use of the principle of the controlled valency.

PTC-resistors the resistance body of which consists of semiconductive barium titanate, the electric resistance of which can increase considerably when the temperature increases to and above the ferro-electric Curie-temperature are known per se. Examples hereof are those resistors the ceramic resistance bodies of which consist of barium titanate in which a part of the barium ions is replaced by  $La^{3+}$  ions or  $Sb^{3+}$  ions or part of the  $Ti^{4+}$  ions by  $Nb^{5+}$  ions.

Applicants have found that PTC-resistors can be manufactured the said temperature-dependence of the electric resistance of which is considerably larger than of known PTC-resistors on the basis of semiconductive titanate.

PTC-resistors manufactured according to the invention show a considerably stronger increase of the electric resistance than the known resistors on the basis of semiconductive barium titanate when the temperature is increased to and above the ferro-electric Curie-temperature, or the absolute increase of the electric resistance in a given temperature range is considerably larger than of those known resistors; often both effects occur in a PTC-resistor obtained with the use of the invention. These PTC-resistors often have a substantially constant temperature coefficient of the electric resistance over a large temperature range.

Consequently, the PTC-resistors according to the invention can advantageously be used in those cases where electric resistors having positive temperature coefficients can be used, for example, for current limiting and stabilization in thermo-regulators and voltage stabilizers, for safeguarding electric motors and for temperature and radiation measurements.

The invention relates to a method of manufacturing a ceramic resistance body consisting of substantially pure semiconductive barium titanate which has been made semiconductive with the use of the principle of the controlled valency from a powder which substantially consists of barium titanate or substantially of compounds which are converted into barium titanate upon heating in an oxygen-containing atmosphere, characterized in that before shaping the powder is intimately mixed with a fluoride of an element of the group consisting of Ca, Sr and Ba in a quantity corresponding to 0.5 - 10 at. percent of fluorine, calculated on barium titanate present in the ceramic resistance body, to a ceramic resistance body thus manufactured and PTC-resistors manufactured by means of said body.

Applicants have found that for the manufacture of PTC-resistors according to the invention the ceramic resistance bodies thereof must consist of substantially pure semiconductive barium titanate and preferably of such a barium titanate which contains a small excess, up to 3 mol. percent and preferably 1.5 - 2.0 mol. percent, of titanium dioxide.

A ceramic resistance body consisting of substantially pure semiconductive barium titanate is to be understood to mean herein such a body which consists for at least 95 mol. percent of barium titanate.

For making barium titanate semiconductive the known methods may be used and at least one element which introduces semiconductivity with the use of the principle of the controlled valency may be incorporated in suitable quantities. Examples of such elements are antimony, bismuth, niobium, cerium, yttrium, rare earth metals, for example, lanthanum.

As a fluoride is preferably used calcium fluoride.

The quantity of fluoride to be used corresponds to 0.5 - 10 at. percent of fluorine, calculated on barium titanate in the ceramic resistance body. This content preferably corresponds to 1 - 8 at. percent of fluorine and in particular to 2 - 6 at. percent of fluorine.

The manufacture of ceramic resistance bodies according to the invention may be carried out, for example, as follows:

Powders of barium carbonate, titanium dioxide and antimony oxide,  $(Sb_2O_3)$  are carefully mixed, for example, by grinding, and the mixture is heated in air at  $1,100^{\circ}\text{C}$  for 60 minutes. The resulting product is ground. The fluoride to be added, for example,  $CaF_2$ , is intimately mixed with the resulting powder, for example, by grinding. The resulting pulverulent product is given the desired shape for example, of a rod, sheet or strip, for example, by compression. The body thus obtained is sintered in an oxygen-containing atmosphere to form a ceramic resistance body, for example, by heating in air at  $1,400^{\circ}\text{C}$  for 60 minutes. The resulting resistance body may be provided in known manner with ohmic electrodes and supply wires for the manufacture of PTC-resistors.

Ceramic resistance bodies to be investigated (wafers, diameter 7.5 mm, thickness 1.85 mm) were provided with ohmic electrodes as a result of which no contact resistances occur. The electric resistance was measured at different temperatures.

In the following table are successively stated the number of the test; the nature and the quantity of fluoride added; particulars, if any, regarding sintering temperature, sintering duration and replacement of part of  $BaO$  by  $SrO$  or of  $TiO_2$  by  $SnO_2$ , respectively; and finally the maximum value of the temperature coefficient of the electric resistivity denoted by  $TC_{max}$ , in per cent per  $^{\circ}\text{C}$ .

The basic composition of the ceramic bodies was the following:

$(BaO)_{1.0} (TiO_2)_{1.0175} (Sb_2O_3)_{0.0015}$ .  
For this composition  $TC_{max} = 38$ . In the table this is stated in experiment Nr. B.

For the definition of the temperature coefficient (TC) of the electric resistivity (R) it holds that:

$$TC = \frac{1}{R} \cdot \frac{dR}{dT} = 2.3 \cdot \frac{d^{10} \log R}{dT} \quad (T, \text{ temperature in } ^{\circ}\text{C})$$

The increase in the electric resistivity at a rise in temperature of  $1^{\circ}\text{C}$  is

$$\frac{R_T + 1}{R_T} = e^{TC}$$

( $e$  = base of natural logarithms.)

For a TC-value of 100 percent per  $^{\circ}\text{C}$ ,  $e^{TC} = 2.78$  which means that per  $^{\circ}\text{C}$  the electric resistance in this case increases by a factor 2.78.

It will be clear that, since with the use of the method according to the invention ceramic resistance bodies can be manufactured which have temperature coefficients of the electric resistivity which are higher than 100 percent per  $^{\circ}\text{C}$ , the increase of the electric resistance at a rise in temperature of  $1^{\circ}\text{C}$  is particularly large in PTC-resistors manufactured from said bodies.

The ceramic bodies according to the present invention are of a fine crystallinity. Applicants suppose that this is due to a limitation of crystal growth by the influence of fluoride. Due to this the bodies show a high breakdown voltage. The high order of reproducibility in the manufacture of the resistors is also due to the said effect.

TABLE

| Test Nr. | Fluoride<br>in mol % | Particulars | TC <sub>max</sub> in<br>% per $^{\circ}\text{C}$ |
|----------|----------------------|-------------|--------------------------------------------------|
| 75 B 1   | 0<br>0.3%; $CaF_2$   |             | 38<br>51                                         |

|    |                       |     |
|----|-----------------------|-----|
| 2  | 1.0%;CaF <sub>2</sub> | 115 |
| 3  | 10%;CaF <sub>2</sub>  | 51  |
| 4  | 1%;CaF <sub>2</sub>   | 21  |
| 5  | as 4                  | 92  |
| 6  | as 4                  | 115 |
| 7  | 1%; CaF <sub>2</sub>  | 92  |
| 8  | as 7                  | 92  |
| 9  | as 7                  | 78  |
| 10 | 1%; CaF <sub>2</sub>  | 92  |
| 11 | 1%; CaF <sub>2</sub>  | 58  |
| 12 | 1%; BaF <sub>2</sub>  | 65  |
| 13 | 1%; SrF <sub>2</sub>  | 68  |

3. The electric ceramic resistor of claim 1 wherein the ceramic body contains 2 to 6 at. percent inclusive of fluoride in the form of fluoride calculated on the barium titanate.
4. The electric ceramic resistor of claim 1 wherein the ceramic body contains 1.5 - 2 mol. percent of titanium dioxide calculated on the barium titanate.
5. In the method of manufacturing a ceramic resistance body consisting of semiconductive barium titanate comprising the steps, first shaping a powder consisting substantially of barium-titanate or compounds heat-convertable to barium titanate and a compound of a metal capable of inducing semiconductivity into the barium titanate into a shaped mass and then sintering the resultant shaped mass by heating in oxygen, the improvement which comprises adding to the powder before shaping at least one fluoride of an element selected from the group consisting of Ca, Sr and Ba in a quantity corresponding to 0.5-10 at. percent of fluorine, calculated on the barium titanate present in the ceramic resistance body.
6. The method of claim 5 wherein the fluoride is employed in an amount corresponding to 1-8 at. percent of fluorine, calculated on the barium titanate present in the ceramic resistance body.
7. The method of claim 5 wherein the fluoride is employed in an amount corresponding to 2-6 at. percent of fluorine, calculated on the barium titanate present in the ceramic resistance body.
8. The method of claim 5 wherein the fluoride is a calcium fluoride.

30

35

40

45

50

55

60

65

70

75

UNITED STATES PATENT OFFICE  
CERTIFICATE OF CORRECTION

Patent No. 3,674,713 Dated July 4, 1972

Inventor(s) JEAN MICHEL BAUDRY GHISLAIN YPERMAN ET AL

It is certified that error appears in the above-identified patent and that said Letters Patent are hereby corrected as shown below:

In the title page:

[72] "yperman" should read -- Yperman --;

"Evere," should be cancelled.

Signed and sealed this 9<sup>th</sup> day of January 1972.

(SEAL)

Attest:

EDWARD M. FLETCHER, JR.  
Attesting Officer

ROBERT GOTTSCHALK  
Commissioner of Patents